

## UNITED STATES PATENT OFFICE.

WILLIAM N. BLAKEMAN, JR., OF MOUNT VERNON, NEW YORK.

## PAINT COMPOSITION.

No Drawing.

Application filed April 16, 1921. Serial No. 461,962.

*To all whom it may concern:*

Be it known that I, WILLIAM N. BLAKEMAN, Jr., a citizen of the United States, and resident of the city of Mount Vernon, in

- 5 the county of Westchester and State of New York, have invented a new and useful Improvement in Paint Compositions, which invention is fully set forth in the following specification.
- 10 The object of this invention is to utilize in the formation of paint composition, the petroleum or mineral oils—especially the heavier distillates and residuals—in conjunction with animal and vegetable drying and
- 15 non-drying fatty oils.

The invention relates particularly to the petroleum or mineral oils obtained chiefly from oil fields in the Appalachian territory, including Pennsylvania, New York, Ohio, 20 Indiana, West Virginia, Kentucky and Tennessee, and from other domestic and foreign oil fields. The oils in this class, or group, of which the Pennsylvania oils are regarded as the type, are known commercially as paraffine base oils, and are regarded chemically as being largely composed of saturated hydrocarbons of the paraffine series. They are soluble in, and miscible with, the various drying, semi-drying, and non-drying fatty oils, but they do not unite chemically with such oils, as when so mixed and then spread on a plain surface, they flow out from such combinations or evaporate, or wash away. This is owing 35 to their indifference to the action of oxygen, all attempts to oxidize them, except at temperatures approaching decomposition or combustion, having failed.

As set forth in my application No. 461,963 filed herewith, I have discovered that these mineral oils of the Pennsylvania type, may be hydrogenated, and that when so hydrogenated they become susceptible to oxidation. And I have further discovered 45 that when so hydrogenated, and particularly if hydrogenated and oxidized, they will unite and form stable and permanent compounds with the animal and vegetable drying, semi-drying and non-drying fatty oils, so that 50 drying-oil-vehicles of any gravity or character desired, may be built up therewith.

Either the crude mineral oil, or any of its fractions, distillates, or residuals, may be employed in carrying out my invention, 55 and by the term mineral oil, or Pennsyl-

vania oil, as used in this specification and in the claims, I intend to include the crude oil, and also its fractions, distillates and residuals.

In demonstration, I select, as being well adapted for use, the distillate now known commercially as "heavy paraffine oil," of .915 sp. gr., and subject it to the action of hydrogen in the presence of catalysts, with heat, until it assumes the color of light vinegar, continuing the operation, if desired, to a light cherry red. This hydrogenated oil may then be mixed with any of the animal or vegetable drying, semi-drying, or non-drying fatty oils, and will unite therewith, 65 the reaction being accelerated by exposure to light, or a gentle heat, or both, and the compound or mixture so formed will, if spread in a thin film on a plain surface, dry and indurate satisfactorily. Thus, a mixture of cotton-seed oil and 20% heavy paraffine oil, hydrogenated, when allowed to blend for 8-10 hours at a gentle heat or 70 in broad sunlight, and spread on a plain surface, will retain its homogeneity, will not 75 break or flow out, and will firm to the touch in 24 hours, with a progressive induration under favorable climatic conditions; whereas, a mixture of an untreated paraffine oil and a fatty oil will fail to show 80 any such result.

After the mineral oil has been hydrogenated, it may be oxidized, if desired, and I have found that such oxidation will greatly accelerate its activity. The oxidation may 90 be effected by heating on oxidizers, a run on the higher oxides of manganese, at a temperature of 185° to 194° Fahr., for one or two hours, being sufficient; and the addition of 2% or 3% of an oxygen-carrier, such as 95 turpentine spirits, will be of marked benefit. If 10% of this mineral oil, hydrogenated and oxidized, be mixed with cottonseed oil, and the mixture, after blending, be spread on a plain surface, it will firm to the touch 100 in 9 hours, and subsequently indurate satisfactorily.

The mineral oil, hydrogenated, or hydrogenated and oxidized, as above described, may be combined with all the drying, semi-drying and non-drying fatty oils in varying proportions from 10% up to 70%, and the drying-oil thus formed will be found very efficacious as a component in all plastic compositions, and will constitute a new ve- 11

hicle for pigments in paints. The gravity of the mineral oil, and the character of the pigment or other solid material used, will govern the proportion required, but a medium percentage of 15% to 20% of the mineral oil will be found to be generally effective.

The fatty oils which fall within the economical scope of my invention and the painting art, at present, are, of the vegetable oils, linseed, tung, cottonseed, soja bean, sunflower seed, cocoanut, palm-kernel, corn, and the like; and, of the marine animal oils, menhaden, fish, seal, whale, porpoise, shark, and the like. These oils may be used, either singly or combined, and, when forming a paint-vehicle with the mineral oil, are preferably used in excess of the latter.

In forming mixtures between the treated mineral oil, and fatty oils, particularly with non-drying fatty oils, I prefer to include a percentage of tung oil, as I have found that its use improves the quality of the mixture and accelerates the firming and induration of the film. The tung oil apparently exerts some peculiar influence in the presence of the mineral oil, as is shown by the fact that if 15% of tung oil be incorporated with a heavy paraffine oil, hydrogenated, and the mixture after blending, without the addition of any other oil, be spread on a plain surface, it will firm to the touch in 4 or 5 hours, and progress to complete induration under favorable conditions, the usual commercial liquid drier hastening the result.

The paint-vehicles which may be formed as a result of my invention, are of universal application, but are especially adapted for use with those anhydrous and inert substances, which, in the present hydrated system of painting, are now used mostly as adulterants or fillers, but which with my new vehicles may be employed as sole body-giving agents, relying upon a moderate percentage of the more expensive metallic oxides and salts for complete opacity in the film. All these substances can be ground in my new vehicles, with great facility, to a smooth, impalpable and emulsive condition; will spread on plain surfaces with beautiful homogeneity and uniformity; will firm to the touch, with a celerity unknown in the painting art; and will indurate to a satisfactory and permanent film. The pigments produced by furnace sublimation of zinc oxide and lead sulphate, now on the market under the name of zinc-lead or leaded zinc, carrying from 5% to 35% lead sulphate, are pre-eminently adapted for use with these vehicles, forming white films, which effectually resist degrading and discoloring weathering effects. Most remarkable combinations may be made also with natural barium sulphate, known commercially as barytes (the ground rock) which for

tinted films, in structural painting, will be found preferable to all other combinations in economy and permanency.

Thus, for example, if a vehicle be formed with 75 parts cottonseed oil, 10 parts heavy paraffine oil, hydrogenated and oxidized, and 15 parts tung oil; or 60 parts cottonseed oil, 25 parts heavy paraffine oil hydrogenated and oxidized, and 15 parts of tung oil; when from 5 to 7 parts of either of these vehicles are properly ground with 10 parts zinc lead (composed of about 65 per cent zinc oxide and 35 per cent lead sulphate) with the usual quantity of commercial turpentine japan drier added, the composition will spread and follow the brush in a smooth and uniform film; firm to the touch in from 1½ to 2 hours, according to climatic conditions, and indurate into a permanent covering. From 5 to 7 parts of such vehicles, properly ground with 15 parts of barytes and 3 parts of zinc-lead of the above composition, and the usual drier, will form a structural covering most economical in manufacture and most resistant to the elements. Not only barytes, but its various manufactured compounds, such as lithopone and the proprietary "whites," can be used as sole body-giving agents, grinding with great facility, even from a granular form, into an impalpable and emulsive condition, showing, when spread as a film, a diffused opalescence in either transmitted or reflected light, the opacity being easily increased by a small percentage of the more expensive metallic oxides and salts.

While my new oil-vehicles, carrying in excess non-drying and semi-drying fatty oils, are particularly adapted for use with anhydrous pigments, and, owing to the low cost of material, will form more economical compositions when so used, they may be used also for hydrated pigments such as Dutch white lead, particularly where the white lead is associated with a metallic oxide or sulphide. Thus, if 7 parts of cottonseed oil carrying 25% heavy paraffine oil, hydrogenated and oxidized, and 15% tung oil, be properly ground with 10 parts of Dutch white lead and 3 parts zinc sulphide, and a drier, the composition, when spread on a plain surface, will, under favorable conditions, firm to the touch in one-half hour and indurate to a satisfactory film.

Although cocoanut and palm-kernel oils are fluid at summer heats, and chill to butters at somewhat lower temperatures, yet when from 10% to 20% of cocoanut oil is used in these new compositions, it will not cloud, flock, or chill out, but will remain in clear solution in the vehicle at temperatures very much below its congealing point; and the presence of this oil or butter in the composition, especially in contact with tung oil, will be found to improve the spreading

power of anhydrous pigments, and the resistance of the film to atmospheric and abrasive influences, without showing a greasy residue or exudation.

5 From 1 to 3 per cent of any of the gums, waxes, resins, petroleum residuals, or like substances, may be added to the compositions, to give an additional resistant effect to the film.

10 Any suitable commercial liquid drier may be employed.

Light, heat, pressure, agitation, and electrical energy may be used whenever deemed advisable.

15 The oil-vehicle herein described, is claimed in my application above referred to.

Having thus fully described my invention, I claim:

1. A paint-composition comprising a mineral oil of the Pennsylvania type, hydrogenated, and a pigment.

2. A paint-composition comprising a mineral oil of the Pennsylvania type, hydrogenated and oxidized, and a pigment.

25 3. A paint-composition comprising a fatty oil; a mineral oil of the Pennsylvania type, hydrogenated; and a pigment.

4. A paint-composition comprising a fatty oil; a mineral oil of the Pennsylvania type, hydrogenated and oxidized; and a pigment. 30

5. A paint-composition comprising tung oil; a mineral oil of the Pennsylvania type, hydrogenated; and a pigment.

6. A paint-composition comprising tung oil; a mineral oil of the Pennsylvania type, 35 hydrogenated and oxidized; and a pigment.

7. A paint-composition comprising tung oil; another fatty oil; a mineral oil of the Pennsylvania type, hydrogenated; and a 40 pigment.

8. A paint-composition comprising tung oil, another fatty oil; a mineral oil of the Pennsylvania type, hydrogenated and oxidized; and a pigment.

9. A paint-composition comprising tung 45 oil, a non-drying fatty oil; a mineral oil of the Pennsylvania type, hydrogenated; and a pigment.

10. A paint-composition comprising tung oil; a non-drying fatty oil; a mineral oil of 50 the Pennsylvania type, hydrogenated and oxidized; and a pigment.

WM. N. BLAKEMAN, JR.